

# United States Patent Office

2,786,733

Patented Mar. 26, 1957

1

2,786,733

## METHOD OF TREATING ABACÁ CORDAGE FIBER WITH THE HYDROLYSIS PRODUCT OF METHACRYLATO CHROMIC CHLORIDE AND PRODUCT PRODUCED THEREBY

George Thomson, Milton, and Chapin A. Harris, Lexington, Mass., assignors to Fabric Research Laboratories, Inc., Boston, Mass., a corporation of Massachusetts

No Drawing. Application September 10, 1953,  
Serial No. 379,463

3 Claims. (Cl. 8—116)

This invention relates to cordage, and more particularly to the modification of abacá fiber for use in cordage.

Abacá fiber, the botanical name of which is *Musa textilis*, is also known as Manila, or Manila "hemp."

Vegetable fibers employed in the manufacture of cordage vary substantially in their physical properties. Generally speaking, the higher the tensile strength of the fiber, the lower is its elongation, which may be illustrated by a comparison between Mexican sisal (*Agave fourcroydes*), also known as henequen, and abacá fiber. Thus, while Mexican sisal may exhibit a tensile strength only three-fourths that of abacá fiber, the elongation of the sisal may be twice that of the abacá. Furthermore, the knot efficiency of Mexican sisal is commonly 1½ times that of abacá fiber, knot efficiency being the ratio of the tensile strength of knotted fiber to the tensile strength of unknotted or straight fiber.

By reason of its generally advantageous properties such as high tensile strength, resistance to abrasion and resistance to deterioration, and notwithstanding its relatively low elongation and knot efficiency, abacá fiber is extensively used in cordage and is probably the most highly regarded vegetable fiber for cordage purposes.

In certain cases, considerations of economy or supply suggest the desirability of blending abacá fiber with other fiber such as Mexican sisal, for cordage purposes. As has been indicated above, sisal has lower tensile strength but higher elongation than abacá fiber. Such blending, however, has not been successful, because when the resulting cordage is subjected to tension, the stress is concentrated in the stiffer and less extensible fiber, namely the abacá fiber. The consequent non-uniform fiber stress results in unsatisfactory rope performance characteristics, including lower tensile and knot strengths.

An object of this invention is to provide abacá fiber of improved characteristics for use in cordage. Another object is to provide a method of producing such improved abacá fiber.

In the accomplishment of the above and other objects, there is provided by this invention modified abacá fiber which exhibits permanent and marked increase of elongation, both in the dry and wet states, and yet exhibits tensile strength comparative to that of the untreated fiber. The increase of elongation may be of the order of several hundred percent; the tensile strength may be decreased somewhat, but such decrease is not of practical consequence in terms of resultant cordage properties.

In producing the modified abacá fiber of this invention, the bond between cellulose cells of the fiber and the middle lamella is relaxed, the middle lamella being the plant material which holds the cellulose cells firmly together. Additionally, cellulose cells are joined or chained sufficiently firmly to maintain high tensile strength of the fiber, and yet sufficiently loosely or slackly to permit increased elongation, the joining or chaining medium being a polymer of the hydrolysis product of methacrylato chromic chloride.

2

In the practice of the invention, the relaxing of the bond between the cellulose cells and the middle lamella, and the chaining or concatenation of the cells by the polymer, may be carried out in the order desired; conveniently, however, the relaxing of the bond between the cellulose cells and the middle lamella is carried out first. In either case, in the resulting modified abacá fiber the bond between cellulose cells and the middle lamella is lax, and the cellulose cells are slackly concatenated by a polymer of the hydrolysis product of methacrylato chromic chloride.

According to a specific illustration of the invention, wherein first the bond between the cellulose cells and the middle lamella is relaxed, abacá fiber is immersed in a 15 12% aqueous solution of sodium hydroxide for a half hour at room temperature, after which the fiber is drained, for example as by centrifuging. The fiber is then washed with dilute (1%) acetic acid to neutralize any residual sodium hydroxide, following which the fiber is rinsed 20 with water, and dried in air.

The action of the sodium hydroxide in the above-described treatment of the abacá fiber evidently is to swell the cellulose cells disproportionately to the middle lamella and thereby weaken or relax the bond between said 25 cells and the middle lamella, but not to destroy said bond. In any event, the effective result is to permit markedly increased elongation of the fiber when it is subjected to tension. It should be pointed out, however, that this treatment alone is not adequate for the purposes of this 30 invention, because of accompanying serious loss of wet strength, namely tensile strength of the fiber when in wet condition.

Continuing with the specific illustration of the invention, the chaining or concatenation of the cellulose cells 35 in the abacá fiber is carried out by first immersing the fiber, previously treated with sodium hydroxide as described above, in a 0.5% aqueous solution of methacrylato chromic chloride at a pH of 4.7. This immersion is continued for a half hour, at room temperature, following which the fiber is drained, and dried in air. Then 40 follows a polymerization step to be described hereinafter.

The structural formula of methacrylato chromic chloride may be shown as



The aqueous solution of methacrylato chromic chloride is highly acidic. Since the abacá fiber is sensitive to strong acid, the solution is partially neutralized by raising the pH thereof to the value of 4.7. This is accomplished by adding an aqueous buffering solution containing 16.5% urea, 5.0% sodium formate, together with 55 sufficient formic acid to bring the buffering solution to pH 6.

Further continuing with the specific illustration, the fiber which has been immersed in the methacrylato chromic chloride solution and dried is then heated in an oven 60 at 325° F. for 20 minutes. The resulting product is the modified abacá fiber of this invention.

During the immersion of the fiber in the methacrylato chromic chloride solution and the subsequent oven heating, there occurs hydrolysis of the methacrylato chromic chloride, polymerization of the hydrolysis product, and 70 attachment of the polymer to cellulose cells of the abacá

fiber. In other words, said cellulose cells are slackly concatenated by a polymer of the hydrolysis product of methacrylato chromic chloride.

Modified abacá fiber produced in accordance with the above specific illustration exhibited highly advantageous properties for cordage purposes. Comparison was made with untreated abacá fiber from the same lot, which exhibited a tensile strength of 5.3 grams per denier and an elongation of 2.3%. On the other hand, the modified fiber exhibited an elongation 2.8 times or 280% that of the untreated fiber, while maintaining comparative tensile strength, namely 95% that of the untreated fiber. Furthermore, the characteristics of the modified fiber were well maintained in the wet condition, the tensile strength being 92% of the dry modified fiber and 87% of the untreated fiber. The elongation of the modified fiber was greater in the wet condition, being 1.3 times that of the dry modified fiber and 3.7 times or 370% that of the untreated fiber.

It will be understood, of course, that the invention is not limited to the details set forth above in the specific illustration. Many variations may be made in carrying out the invention, depending upon particular conditions and the results desired in individual cases. Certain of such variations are herein suggested. Thus, in alkali metal hydroxide treatment to relax the bond between cellulose cells and the middle lamella of the abacá fiber, other alkali metal hydroxides such as potassium hydroxide may be employed in place of sodium hydroxide.

In the sodium hydroxide treatment of abacá fiber disclosed hereinabove, the concentration of sodium hydroxide in the aqueous solution may be varied, but generally speaking, concentrations less than 10% are ineffective, and concentrations above 15% afford no particular advantage. The temperature of the sodium hydroxide solution may vary in the general range of 0° to 30° C. The solution at 10° C. is highly effective, but cooling is ordinarily required, and temperatures above 20° C. do not provide additional benefits. The time of treatment may be as short as 5 to 10 minutes; 20 minutes is highly advantageous; 30 minutes is commercially a practical optimum; and generally speaking, with times substantially longer than about 30 minutes the effectiveness of the treatment is diminished.

In the methacrylato chromic chloride treatment of the abacá fiber, which has been specifically illustrated hereinabove, the concentration of the aqueous methacrylato chromic chloride solution, in which the fiber is immersed, may vary from about 0.25% to about 1%. Concentrations above 1% are of decreasing effectiveness. The time of immersion of the fiber in the methacrylato chromic chloride solution may vary from about ½ hour, which is adequate, to over 20 hours. The pH of the solution may vary from about 3 to about 5, depending in part upon the temperature at which the fiber subsequently is to be oven-heated. Thus, if the oven-heating is to be carried out about 200° F., a solution pH of about 4 is desirable, whereas a pH nearer 5 is advantageous when the oven-heating is to be carried out in the range of 300° to 350° F.

For the concatenation of cellulose cells in the abacá fiber, the hereinabove-described treatment is preferred wherein the fiber is immersed in aqueous methacrylato chromic chloride solution, and the fiber subsequently oven-heated. However, an alternative treatment with methacrylato chromic chloride may be employed. According to this alternative treatment, the dilute aqueous methacrylato chromic chloride solution, before partial neutralization, is brought to a temperature of about 200° F. and allowed to cool. Following the immersion of the fiber in the methacrylato chromic chloride solution, the fiber is dried at room temperature without subsequent oven-heating. The heating of the dilute methacrylato chromic chloride solution appears to bring about or initiate hydrolysis of the methacrylato chromic chloride and polymerization of the hydrolysis product such that concatenation of cellulose

cells of the immersed fiber is accomplished at room temperature. Of course it will be understood that this alternative treatment of the fiber might still be followed, in certain instances, by oven-heating of the treated fiber.

While in the practical accomplishment of the invention, it is preferred first to carry out the sodium hydroxide treatment of the abacá fiber, followed by the methacrylato chromic chloride treatment, these treatments may be carried out in the reverse order. In other words, as has been previously suggested, the relaxing of the bond between the cellulose cells and the middle lamella, and the concatenation of cellulose cells may be carried out in either sequence.

It will be understood that the invention may be carried out to provide, within limits, modified abacá fiber of selected increased elongation, for example, to match the elongation properties of other varieties of fiber with which it may be desired to blend the abacá fiber in the manufacture of cordage.

The utilization of modified abacá fiber of this invention in cordage makes possible the imparting of highly advantageous characteristics thereto, such as higher impact resistance, or as technically known, higher energy absorption. This characteristic is exhibited, for example, when a rope becomes taut in commencing the towing of a boat. Fiber of this invention further makes possible improved flex abrasion of cordage, exhibited in greater durability and resistance to wear; and better translation of fiber strength to cordage, because of improved distribution of stresses and relief of stress concentration. Furthermore, by reason of the permanent modification of the fiber afforded by this invention, improvement persisting throughout repeated mechanical stressing of cordage is made possible.

It will be seen that by the present invention abacá fiber may be utilized to increased advantage in the manufacture of cordage, and effective blending of abacá fiber with fibers of other varieties may be accomplished.

It will be understood that various modifications may be made while still coming within the scope of the invention.

Having disclosed our invention, what we claim as new and desire to secure by Letters Patent of the United States is:

1. The method of producing cordage fiber of high elongation from abacá fiber which comprises immersing said abacá fiber in a 10-15% aqueous solution of an alkali selected from the group consisting of sodium hydroxide and potassium hydroxide for about 5-30 minutes at a temperature of about 0-30° C., draining said fiber, neutralizing residual alkali and washing said fiber with water, drying said fiber, immersing said fiber in a 0.25-1% water solution of methacrylato chromic chloride of pH about 3-5 at room temperature for about ½-20 hours, draining said fiber and drying it, and heating the thus-treated fiber at about 300-350° F. for a time in the neighborhood of 20 minutes.

2. As a new and useful product, cordage fiber of high elongation produced from abacá fiber by immersing said abacá fiber in a 10-15% aqueous solution of an alkali selected from the group consisting of sodium hydroxide

and potassium hydroxide for about 5-30 minutes at a temperature of about 0-30° C., draining said fiber, neutralizing residual alkali and washing said fiber with water, drying said fiber, immersing said fiber in a 0.25-1% water solution of methacrylato chromic chloride of pH about 3-5 at room temperature for about ½-20 hours, draining said fiber and drying it, and heating the thus-treated fiber at about 300-350° F. for a time in the neighborhood of 20 minutes.

3. The method of producing cordage fiber of high elongation from abacá fiber which comprises immersing said abacá fiber in a 12% aqueous solution of sodium hydroxide for about one-half hour at room temperature, draining said fiber, neutralizing residual sodium hydroxide with acetic acid and washing said fiber with water, drying

said fiber, immersing said fiber in a 0.5% water solution of methacrylate chromic chloride of pH about 4.7 at room temperature for about one-half hour, and heating the thus-treated fiber at 325° F. for 20 minutes.

**References Cited in the file of this patent****UNITED STATES PATENTS**

2,273,040 Iler Feb. 17, 1942

2,524,803 Iler Oct. 10, 1950  
2,544,666 Goebel et al. Mar. 13, 1951  
2,549,220 McLaren Apr. 17, 1951

**OTHER REFERENCES**

5 Textile Research Journal, October 1951, pp. 740-746,  
(Copy in P. O. Libr.)